

# United States Patent Office

2,876,199

Patented Mar. 3, 1959

1

2,876,199

## LUBRICANTS

Jones I. Wasson and William C. Howell, Jr., Union Township, Union County, N. J., assignors to Esso Research and Engineering Company, a corporation of Delaware

No Drawing. Application April 22, 1955

Serial No. 503,326

3 Claims. (Cl. 252—55)

This invention relates to open gear lubricating compositions. Particularly, the invention relates to improved open gear lubricants which comprise mixtures of asphaltic materials and highly aromatic solvent-extract oils having low viscosity indices and low aniline points.

In the past, gear lubricants have been made from blends of asphaltic materials and mineral oils. The asphaltic materials used have been generally selected from a wide range of petroleum crude oil residua and the mineral oil components of the blend have been usually of the mixed base or naphthenic type. The viscosity of the diluent oils have ranged from about 60 to about 300 SUS/210° F.

It has not been hitherto appreciated that the type and viscosity index of diluent oil used in the manufacture of open gear lubricants was of any importance. It has now been discovered, however, and forms the object of this invention that superior gear oils are obtained from blends of asphalts with diluent oils having a high aromatic content, particularly those having aniline points from about 80° to about 120° F. and viscosity indices below about 0. It has been found that these aromatic type oils have excellent solvent properties for asphalts and the blends approach true solution. This is in contrast to the gels or semi-gels obtained upon blending asphalt or asphaltic materials with relatively high viscosity index oils having low solvent properties for asphalts.

The blends prepared in accordance with this invention give outstanding lives on open gears, which is believed to be due to the unusual metal-adhering properties and to their ability to maintain lubricant films on working parts because of their superior fluidity and stringiness. These properties of improved metal adherence and superior fluidity or solution properties are obtained by use of the particular diluent oils, which is the gist of the inventive concept.

The invention will be more clearly explained by reference to the following examples:

## EXAMPLES 1-16

To illustrate the invention, 16 experiments were performed using different asphaltic materials and different

2

diluent oils. Two types of asphalts were used. Asphalt A was a reduced asphalt from a Talco crude oil and asphalt B was a reduced and oxidized Venezuelan asphalt. Six different diluent oils were used. The inspection test results on these diluent oils are set out in Table I below:

Table I.—Diluent oil inspections

| 10 | Designation | Gravity | Vis./210° F.<br>(SUS) | V. I. | Aniline<br>Point<br>(°F.) |
|----|-------------|---------|-----------------------|-------|---------------------------|
| 15 | Oil A       | 0.9410  | 73                    | 17    | 218                       |
|    | Oil B       | 0.9330  | 73                    | 49    | 190                       |
|    | Oil C       | 0.9705  | 73                    | -48   | 97                        |
|    | Oil D       | 0.9818  | 59                    | -115  | 88                        |
|    | Oil E       | 0.9883  | 143                   | -235  | 111                       |
|    | Oil F       | 0.9982  | 358                   | -330  | 118                       |

Diluent oils A and B represent the prior art diluent oils. It will be noted that they have viscosity indices of 17 and 49, respectively, and aniline points of 218° and 190° F., indicating a low aromatic content. Diluent oils C-F are highly aromatic extracts from mineral oils. Diluent oil C is an extract obtained by the silica gel extraction of a distillate, whereas diluent oils D, E, and F were obtained by phenol extraction. It will thus be seen that blends prepared from either asphalt A or B with diluent oils A and B represent the prior art gear lubes, whereas with diluent oils C-F blends are prepared in accordance with the inventive concept.

Various proportions of the asphalts and diluents described above were blended by admixing the two chosen materials and heating with agitation until solutions were obtained. This method of preparation of the gear lubricants is well known to the prior art and forms no part of the inventive concept.

These open gear lubricants were submitted to a gear rig test which has been designed to test the lubricating life of an open gear lubricant. The test may be generally described as follows:

40 A 32-inch pitch diameter cast iron gear is driven by means of a 4-inch pinion gear which is connected to an electric motor. The 32-inch gear is connected to a dynamometer for measuring the gear load. The gears are lubricated with the lubricant to be tested and are run 45 at a temperature of from 80° to 90° F., at uniform pinion gear speed of 400 R. P. M., and a load of 750 lbs. per tooth until the lubricant wears off the gear teeth and exposes free metallic surfaces. The hours to exposure of free metal is reported as the lubricating life of the lubricant.

The results of subjecting the open gear lubricants of Examples 1-16 to this test are set out in Table II below.

Table II.—Gear rig test results

| Ex. No. | Asphalt (wt. percent) |      | Diluent Oil (wt. percent) |      |      |      |      |   | Blend Vis.<br>(SUS/<br>210° F.) | Gear Rig<br>Life, Hrs. |
|---------|-----------------------|------|---------------------------|------|------|------|------|---|---------------------------------|------------------------|
|         | A                     | B    | A                         | B    | C    | D    | E    | F |                                 |                        |
| 1       | 62.4                  | 37.6 |                           |      |      |      |      |   | 1,451                           | 8.0                    |
| 2       | 58.5                  |      | 41.5                      |      |      |      |      |   | 1,402                           | 3.0                    |
| 3       | 55.0                  |      |                           | 45.0 |      |      |      |   | 1,468                           | 16.0                   |
| 4       | 40.0                  |      |                           |      |      |      | 60.0 |   | 1,472                           | 12.8                   |
| 5       | 52.0                  |      |                           |      |      | 48.0 |      |   | 1,464                           | 19.5                   |
| 6       | 58.0                  |      | 42.0                      |      |      |      |      |   | 1,837                           | 5.7                    |
| 7       | 58.0                  |      | 42.0                      |      |      |      |      |   | 2,128                           | 2.0                    |
| 8       | 60.0                  |      |                           | 40.0 |      |      |      |   | 1,935                           | 21.0                   |
| 9       | 58.0                  |      |                           | 42.0 |      |      |      |   | 2,048                           | 15.0                   |
| 10      | 65.0                  |      | 35.0                      |      |      |      |      |   | 2,460                           | 4.0                    |
| 11      | 58.0                  |      |                           |      |      | 42.0 |      |   | 2,594                           | 17.8                   |
| 12      | 48.0                  |      |                           |      |      |      | 52.0 |   | 2,390                           | 16.0                   |
| 13      | 71.0                  |      | 29.0                      |      |      |      |      |   | 5,037                           | 5.0                    |
| 14      | 58.0                  |      |                           |      |      |      | 42.0 |   | 4,207                           | 11.4                   |
| 15      | 72.0                  |      |                           |      | 28.0 |      |      |   | 4,630                           | 18.0                   |
| 16      | 68.0                  |      |                           |      |      | 32.0 |      |   | 5,509                           | 24.0                   |

An examination of the data of Table II shows the outstanding advantage of the gear lubes of this invention.

In Examples 1-5, blends having comparable viscosities below about 1500 SUS/210° F. are compared. Examples 1 and 2 represent prior art blends and Examples 3-5 represent blends prepared in accordance with the invention. Examples 6-9 compare prior art blends, Examples 6 and 7, to the inventive blends, Examples 8 and 9, at the 2000 viscosity level. The advantages of the latter are obvious. In Examples 10-12, blends at the 2500 viscosity level are compared, and in Examples 13-16, blends at the 4,000-5,000 viscosity level are compared. An outstanding advantage is shown at both these viscosity levels for the gear lubricants of this invention.

#### ASPHALTIC MATERIAL

The asphaltic materials which are operable in the concept of this invention may be any of the asphalts obtained from petroleum crude oils by processes known to the art. For example, those petroleum crudes having high asphaltic contents such as those of South America, for example, Lagunillas; California, such as San Joaquin; or Mid-Continent crudes, may be used as the source for the asphaltic material. The petroleum crude oils are treated for removal of the lighter fractions by well-known methods, for example, steam distillation, vacuum flashing, or by solvent separation, e. g., butane or propane de-asphalting.

It may also be desirable to oxidize the asphaltic materials obtained from the reduction of the petroleum crude by blowing with air or by any other means known to the art. As has been described before, oxidation of these asphaltic materials improve their properties of ductility, increase their softening point, and reduce their brittleness.

The asphaltic constituent of the blends of the invention may also be prepared by cutting back a heavy asphalt with a mineral oil to reduce the viscosity of the asphalt to one within the desired range.

In addition to the petroleum asphalts mentioned above, natural asphalts, such as Trinidad, Bermudez, Gelsonite, Grahamite, or Cuban may be used. Blends of these natural-occurring asphalts with petroleum asphalts may also be used.

The asphaltic material operable in the concept of this invention may be any of the above-described natural or petroleum asphalts having viscosities in the range of from 200 to 2,000 Saybolt Furol at 300° F. Preferred, however, and contemplated in the preferred embodiment of this invention are those petroleum asphaltic materials having viscosities from about 240 to about 1200 Saybolt Furol at 300° F.

#### DILUENT OIL

As was stated above, the gist of the instant invention lies in the discovery that a diluent oil of low viscosity index and high aromatic content has greater solvent power for the asphaltic component of the blend. The diluent oils chosen will have viscosities at 210° F. within the range of from about 60 to about 360 SUS and will have aniline points (descriptive of the aromatic content) within the range of from about 80° to about 120° F. The viscosity indices of these solvent extracts will be between about -40 and about -350.

These highly aromatic solvent extracts are obtained from naphthenic base oils such as coastal distillates, by solvent extraction procedures which are known to the art such as phenol extraction, silica gel extraction, and the like. A preferred method of preparing a suitable diluent oil is by phenol extraction of a coastal distillate. It will be understood, of course, that mixtures of these diluent oils may be used.

#### ADDITIVE MATERIALS

The improved gear lubricants of this invention comprise the blend of an asphaltic material such as a petroleum asphalt and a highly aromatic diluent oil. It

should be understood, however, that other additive materials may be blended with these components to improve the final characteristics of the blend. For example, tackiness of the lubricant may be improved by adding to the blend from 1 to 5 wt. percent of high molecular weight polymers and copolymers such as polyisobutylene, copolymers of isobutylene and styrene, and the like.

For example, a blend of 45.0 wt. percent of asphalt A with 55.0 wt. percent of diluent oil C containing 2.16 wt. percent of a polyisobutylene of 21,000 mol. wt., Staudinger, gave a gear rig test life that was 2.5 hours longer than the same blend without the polyisobutylene. In another example, a blend of 46.0 wt. percent of asphalt B and 53.5 wt. percent of diluent oil C containing 0.5 wt. percent of a polymer of isobutylene and styrene having a styrene content of 50% had a gear rig life of more than 36 hours.

It is also contemplated that volatile solvents may be added to the gear lubricants of this invention to reduce their viscosity temporarily for purposes of application. These volatile solvents such as 300°-500° F. boiling range petroleum distillates and chlorinated hydrocarbons, e. g., trichloroethylene, etc., evaporate after application, leaving a film of higher viscosity material deposited upon the metal surfaces to be lubricated.

#### PROPORTIONS

The proportions used to prepare the open gear lubricants of this invention will depend upon the viscosity of the starting materials and the viscosity desired in the final blend. Ordinarily, however, it is desired that the final lubricant have a viscosity between about 1,000 and 6,000 SUS at 210° F. for best lubricating results. Thus, from about 20 to about 90 wt. percent of the asphalt may be blended with about 80 to about 10 wt. percent of the diluent oil. A preferred range, and one operable with most asphaltic materials and diluent oils will be between about 40 to 70 wt. percent of the asphalt with about 60 to 30 wt. percent of the diluent oil.

The amount of additive materials blended with the gear lubricants will also depend upon the characteristics of the desired final product. Ordinarily, from about 0.2 to about 5.0 wt. percent of such additives as polymers of isobutylene and copolymers of isobutylene with other polymerizable monomers may be used. A preferred range is about 0.6 to about 3.0 wt. percent.

The volatile solvent may be used in amounts varying between about 5.0 and 20.0 wt. percent, preferably about 10.0 to about 15.0 wt. percent.

To summarize briefly, this invention relates to improved open gear lubricants which comprise an asphaltic material such as a reduced or reduced and oxidized asphalt blended with a diluent oil which is highly aromatic in nature and which has a viscosity index between about -40 and -350 and an aniline point of about 80° to about 120° F. The diluent oil is preferably phenol extract from a coastal distillate, having a viscosity index of about -40 to about -330, a viscosity of 210° F. of about 60 to 360 SUS, and an aniline point of between about 90° and about 120° F.

The improved open gear lubricants of this invention may contain minor amounts of additive materials known to the art without departing from the spirit thereof. Volatile solvents such as trichloroethylene, petroleum solvents, and similar materials may also be contained in the final formulation.

What is claimed is:

- An improved open gear lubricant having a viscosity of 1,000 to 6,000 SUS at 210° F. consisting essentially of a blend of from about 40 to 60 wt. percent of an asphaltic material selected from the group consisting of reduced and reduced and oxidized asphalts with about 60 to 30 wt. percent of a highly aromatic solvent extract oil, said extract oil having a viscosity of 210° F. of about 60-360 SUS, a viscosity index of from about -40 to -330 and

an aniline point between about 90° and 120° F., percentages being by weight based on the weight of the total composition.

2. An improved gear lubricant according to claim 1 which contains combined therein about 0.6 to 3.0 wt. percent of a polymer of styrene and isobutylene having a styrene content of about 50%.

3. An improved open gear lubricant having a viscosity of about 5,500 SUS at 210° F. consisting essentially of a blend of from about 68 wt. percent of a reduced and oxidized asphalt with about 32 wt. percent of a highly aromatic phenol extract of a naphthenic distillate having a viscosity of 143 SUS at 210° F., a viscosity index of about -235 and an aniline point of about 111° F.

## References Cited in the file of this patent

## UNITED STATES PATENTS

|           |                        |               |
|-----------|------------------------|---------------|
| 2,211,921 | Brunstrum et al. ----- | Aug. 20, 1940 |
| 2,274,749 | Smyers -----           | Mar. 3, 1942  |
| 2,488,293 | Hoiberg -----          | Nov. 15, 1949 |
| 2,607,732 | Duchon -----           | Aug. 19, 1952 |
| 2,607,733 | Oberlink -----         | Aug. 19, 1952 |

## OTHER REFERENCES

10 "Motors Oils," by Georgi, Reinhold Pub. Co., 1950, pp. 153-155.